

# UNITED STATES PATENT OFFICE.

JULIUS H. HOELSCHER, OF CHICAGO, ILLINOIS

## WATERPROOFING PRESERVATIVE DRESSING.

No. 923,176.

Specification of Letters Patent.

Patented June 1, 1909.

Application filed June 17, 1908. Serial No. 438,952.

*To all whom it may concern:*

Be it known that I, JULIUS HENRY HOELSCHER, a citizen of the United States, and a resident of the city of Chicago, in the county 5 of Cook and State of Illinois, have invented certain new and useful Improvements in Waterproofing Preservative Dressing, of which the following is a specification.

This invention has for its object the preparation of a fluid dressing adapted for application to leather of any kind or to fabric to render the same water proof and to preserve the same.

It is an object of this invention to provide 15 a fluid dressing adapted to permeate the leather or fabric to which applied to fill or partly fill the intercellular spaces, capillary fibers and the interstices therein with an elastic substance of slightly oily nature 20 which resists the penetration of water.

It is a further object of the invention to provide a water proofing dressing and preservative adapted to maintain its fluidity at any atmospheric temperature and which 25 maintains the articles to which applied in a soft and pliable condition.

Finally it is an object of the invention to afford an antiseptic water proof dressing of such a nature as to be immediately absorbed 30 in the material to which applied leaving the surface thereof in a condition to receive a polish or other treatment should it be desired.

It is also an object of the invention to provide a transparent, colorless dressing which 35 will not affect the color of the article to which applied.

The invention consists in the matters hereinafter described and more fully pointed out and defined in the appended claims.

40 In preparing the dressing a gum or resin is mixed with an oil and with alcohol or a fluid adapted to assist in cutting the gum, in proportions adapted to form a relatively thin fluid. For this purpose I prefer to use sandarac resin as the gum, though other gums or resins might be substituted. This is cut with alcohol of any kind though conveniently wood alcohol may be used, and to this an oil, preferably a vegetable oil, such as castor oil is added to afford a solution in which 45 sufficient of the oil is taken to hold the gum in a semi-fluid or viscous condition after the evaporation of the alcohol.

One satisfactory preparation is provided 55 by using approximately three pounds of sandarac resin, five gallons of castor oil and ten

gallons of alcohol. The resulting thin and slightly viscous fluid is then bottled or placed in hermetically sealed cans and retains its fluidity and may be applied at any atmospheric temperature.

In applying (as for example to shoes of any kind) the preparation may be spread by means of a brush very freely into and upon the seams and soles, a thinner coating applied to the upper of the shoe, the dressing immediately is absorbed leaving the surface dry but filling the intercellular spaces with the dressing. As the alcohol evaporates, the remaining composition of matter assumes a greater density and viscosity though the presence of the oil maintains the same in a semi-fluid and slightly oily condition, and rendering the leather very soft and pliable, effectually excluding water.

In practice, it has been found that even canvas shoes treated with this preservative dressing effectually shed water without injury to the appearance of the shoe. When used for water proofing fabrics as a substitute for "oil skins" or for use as tarpaulins or for any other purposes, the nature and fluidity of the preparation are such that the capillary fibers of the fabric take up the preparation very rapidly retaining the same 85 therein and being somewhat distended by the same, thus filling the interstices and rendering the same water proof. The slightly oily nature of the material, after the evaporation or partial evaporation of the alcohol, prevents the adhesion of moisture to the fabric, thus preventing the penetration of the fabric thereby, though such oily texture is not sufficient to be distinguishable to the touch or to soil or injure any fabric brought in contact with the water proofed garment.

The elasticity of the dressing serves to render the fabric in a soft and pliable condition, and inasmuch as all the ingredients are antiseptic in their character, a perfectly 90 sanitary dressing is secured and one that will not deteriorate in any climate or under any natural conditions.

Of course, I am aware that other ingredients may be added if preferred, the proportion may be varied. These in some instances, however might render the article treated unsightly and in some instances might prevent the leather or fabric from perfectly absorbing the dressing thus losing a very 105 important feature of this invention, namely, that the dressing does not affect color and

when applied is quickly absorbed leaving but very slight visible trace, if any.

Inasmuch, as changes in ingredients and proportions may be varied, I do not purpose limiting this application for patent otherwise than necessitated by the prior art.

I claim as my invention:

1. An antiseptic and preservative water proof dressing comprising less than five per cent. gum, a more or less volatile liquid to cut the same and a vegetable oil of substantially one-half the quantity of the volatile liquid mixed therewith to afford in connection with the gum an elastic and slightly oily medium adapted to be retained in the interstices in the articles to which applied after the evaporation of the cutting fluid therefrom.

2. A water proofing and preservative dressing consisting of a small per cent. of sandarac resin, castor oil and alcohol in proportion approximately one to two, and said ingredients affording a thin, transparent, colorless fluid.

3. A preparation of the class described consisting approximately of three pounds of sandarac resin, five gallons of castor oil and ten gallons of alcohol.

In testimony whereof I have hereunto subscribed my name in the presence of two subscribing witnesses:

JULIUS H. HOELSCHER.

Witnesses:

C. W. HILLS,  
K. E. HANNAH.